# EUROPEAN PATENT SPECIFICATION

(11) **EP 0 029 234 B1**
(45) Date of publication and mention of the grant of the patent: **09.11.1983**
(21) Application number: 80107059.0
(22) Date of filing: 14.11.1980
(51) Int. Cl.: H01B 7/02, H01B 3/44, B32B 27/08

(54) **Low voltage cable provided with improved insulating layer**
Niederspannungskabel mit Isolierschicht
Câble à basse tension muni d'une gaine d'isolation

(30) Priority: 15.11.1979 IT 2729579
(43) Date of publication of application: 27.05.1981
(73) Proprietor: SOCIETA CAVI PIRELLI S.p.A., 20123 Milano (IT)
(72) Inventor: Beretta, Germano, Monza (Milan) (IT)
(74) Representative: Gernhardt, Claus, Dipl.-Ing.

## Description

The present invention concerns an improvement to low voltage cables wich comprise a single conductor and which are insulated with a material based on polyvinylchloride (PVC), said cables being well known as wiring cables for civil appliances.

In the state of the art these cables are generally realized taking into account especially very low costs yet compatibility with the electrical, mechanical and ageing characteristics, determined by standards in force.

It follows that the insulating layer of the wiring cables for civil appliances is always realized with materials having a very high mineral filler content up to 30 parts by weight per 100 parts by weight of resin.

The insulating layer of low voltage cables used up to now had always a quite rough surface owing to the high content of mineral fillers. The high friction coefficient due to the roughness creates difficulties during drawing, and abrasions because of the contact with the inner surface of the conduits. Moreover, in spite of the presence of the mineral filler the content of polyvinylchloride is always high with respect to said mineral filler. The polyvinylchloride is a thermoplastic material and in case of overheating it melts, exposing the conductor, with serious risk of short circuits.

There is also known a flame-resisting electrical cable (DE―B―2 051 192) having a conductor constituted by one wire or more wires stranded together and covered with an insulating layer and with an outer layer, both layers being made from a material based on polyvinylchloride (PVC), and containing at least a plasticizer, said material for the insulating layer containing also at least a mineral filler. In order to obtain high flame-resistance the materials forming the insulating and/or the outer layer contain from 6 to 40 percent by weight of magnesium carbonate on the total quantity of the material and at least 20 percent by weight of a chlorinated substance and from 1 to 15 percent by weight of antimony trioxide.

The present invention aims to improve with the electrical characteristics being the same, any other properties of the wiring cables for civil appliances used up to now, eliminating the drawbacks, but retaining very low costs of the product.

The said aim is accomplished by the present invention by providing a low voltage cable having a conductor constituted by one wire or more wires stranded together and covered with an insulating layer and with an outer surrounding layer, both layers being made from a material based on polyvinylchloride (PVC), and containing at least a plasticizer, said material for the insulating layer containing also at least a mineral filler, which is characterized by the fact that said mineral filler is contained in the material for the insulating layer in a proportion from 40 to 500 parts by weight per 100 parts by weight of polyvinylchloride, said plasticizer is contained in the material in a proportion from 60 to 120 parts by weight per 100 parts by weight of polyvinylchloride, said outer layer being a skin for the surface of said insulating layer and having a thickness from 5 to 30 percent of the thickness of said insulating layer, the material constituting said skin containing a quantity of plasticizer from 10 to 40 parts by weight per 100 parts by weight of polyvinylchloride.

The invention teaches a cable the insulating layer of which, even if it comprises a high mineral filler content, much higher than the presently used content, has such a structure as to offer good mechanical characteristics, a very low friction coefficient, and a high fire resistance. Furthermore said insulating layer can be easily stripped and therefore easily applied and permits a high reliability in case of overheating.

The enclosed drawing illustrates by way of a non-limiting example a practical embodiment of the invention:
Figure 1 shows schematically a perspective view of a length of a cable according to the invention.
Figure 2 shows a test path for wiring cables of civil appliances.

The low voltage cable 10 shown in figure 1 comprises a conductor 11 constituted by a single wire, but it is understood that said conductor 11 could also comprise a plurality of wires stranded together.

The conductor 11 is covered with an insulating layer 12 extruded thereon.

The insulating layer 12 is constituted by a material based on polyvinylchloride (PVC), containing at least a plasticizing mineral filler.

The mineral filler in the material is present in a proportion from 40 to 500 parts by weight per 100 parts by weight of polyvinylchloride (PVC).

Among the substances which can be added to the material as a mineral filler the following are preferable:
- calcium carbonate in a preferred proportion of 400 parts by weight per 100 parts by weight of PVC;
- magnesium carbonate in a preferred proportion of 400 parts by weight per 100 parts by weight of PVC;
- calcined kaolin in a preferred proportion of 300 parts by weight per 100 parts by weight of PVC.

The material of the insulating layer further contains a plasticizer in a proportion from 60 to 120 parts by weight per 100 parts by weight of PVC.

In a preferred embodiment, the plasticizer is contained in a quantity of 100 parts by weight per 100 parts by weight of PVC.

The insulating layer 12 is covered on its surface with a skin 13 or thin layer which is constituted by a material based on PVC and containing at least a plasticizer.

Preferably, the plasticizer is Di-2-(ethylhexyl)phthalate (D.O.P.).

The content of plasticizer contained in the skin 13 is 10 to 40 parts by weight per 100 parts by weight of PVC. Its preferred content is 30 parts by weight per 100 parts by weight of PVC.

The thickness of the skin 13 is small with respect to the thickness of the insulating layer. The skin thickness might be comprised between 5 and 30% of the insulating layer thickness and preferably is 15% of the same.

Surprisingly it has been noted that, even if the material of the insulating layer 12 is ultra- loaded, the structure of the cable 10 inclusive of skin 13 has a resistance to tensile stresses sufficient for the handling of the cable since the mechanical stresses occuring for example during the winding on the drum are taken up prevalently by the skin 13.

The electrical characteristics of said cable are good.

The outer surface of the cable 10 is moreover very smooth and very bright, owing to the prevalent presence of PVC in the skin 13, so that the cable 10 has a very low friction coefficient at its outer surface in respect to that of cables in use up to now. Said smoothness and brightness permit the drawing of the cable inside the conduits with easy, gentle and continuous sliding.

Another advantage offered by the cable 10 is the ease of stripping of the conductor 11, so that the insulating layer can easily and completely be removed from the conductor during the connecting and sealing operations.

In fact, it is sufficient to cut circularly the skin 13 and the insulating layer 12 down to the conductor 11 to remove a hollow pin comprising the skin 13 and the underlying insulating layer 12 to which the skin 13 adheres perfectly because it is constituted by a material having the same base of PVC. The hollow pin cavity corresponds to the space previously occupied by the conductor 11.

In a cable according to the invention, in case of overheating, any melting of the PVC will never expose the conductor 11, owing to the presence of a high mineral filler content which filler remains compact, preventing the melted PVC from draining and on the contrary keeping the latter in place.

Moreover, the fact that a cable 10 according to the invention comprising an insulation with a high content of mineral filler has always a sufficiently high plasticizer-resin ratio, contributes to give the cable 10 itself a good cold flexibility.

A further property of cable 10 is a good behaviour to thermocompression because of the essentially "mineral" structure of the material.

Said structure, shown by a material with high mineral filler content, improves also the thermal conductivity of the cable 10 with respect to conventional materials. It follows a more rapid cooling of the cable.

Moreover, in contrast to conventional wiring cables, the material according to the invention does not include any colouring pigments, especially in the insulating layer, with a minimum risk, therefore, of decay of the insulating characteristics.

Moreover, the presence of a high mineral filler content makes the cable 10 particularly resistant to flames since said high quantity of filler, besides being incombustible, improves the compatibility of PVC resin with chloroparaffins.

A cable 10 has a further advantage resulting from the good impermeability of skin 13, which lowers greatly the absorption of water of the assembly.

The advantages of the invention are still more evident from the results obtained with a cable having a conductor of 1,41 mm in diameter, coated with a covering having a thickness S=0,7 mm, where S=S,+S_{P=}0,6 mm+0,1 mm, where Sᵢ=insulating layer thickness and Sp=skin thickness.

The materials used for realizing the skin 13 and the insulating layer 12, respectively, are described herebelow:

Tests conducted on said cable gave the following results:
- electrical characteristics: insulation resistance of 0,2 MΩ/km, measured under water at 70°C;
- flame resistance: "oxigen index" of 28. The test was conducted with the ASTM D 2863-70 method, on the cable after having removed the conductor;
- cold flexibility: the tests were conducted according to standards CEI 20-11 Quality R issue 1968. This latter test was chosen since it is one of the most severe among the standardized tests;
-very low friction coefficient: it had been measured the force F necessary to draw a bundle of three cables along a conventional corrugated PVC tube, for a path (see Figure 2) presenting three angles, α, β, γ, where α=β=90° and γ=135°. α is the angle comprised between 1₁ and I₂, 13 is the angle between 1₂ and 1₃ and y the angle between 1₃ and l₄. The angles α and β were radiused according to an arc of circle having radius r=10 cm. Each of the three cables had the following dimensional characteristics:
- conductor diameter=1,41 mm
- insulating layer plus skin thickness=0,7 mm (insulating layer thickness=0,6 mm, skin thickness=0,1 mm).

The force necessary for the drawing is F=2,5 kg. The advantage is considerable if it is considered that to draw a bundle of cables, with dimensions equal to those of the bundle on which the experimental tests have been conducted, but realized with two cables of conventional type, it is necessary to apply a drawing force of 9 kg.
- absorption: the said cable was kept under water at 100° during 24 hours. At the end of this period it had been found an absorption of 10 mg/cm², a value to be considered extremely satisfactory for a cable having such a high content of mineral filler in its insulation.

The particulars of practical realization of the invention can change according to needs, but all will be included in the scope of the invention.

## Claims

1. Low voltage cable having a conductor constituted by one wire or more wires stranded together and covered with an insulating layer and with an outer surrounding layer, both layers being made from a material based on polyvinylchloride (PVC), and containing at least a plasticizer, said material for the insulating layer containing also at least a mineral filler, characterized by the fact that said mineral filler is contained in the material for the insulating layer (12) in a proportion from 40 to 500 parts by weight per 100 parts by weight of polyvinylchloride, said plasticizer is contained in the material in a proportion from 60 to 120 parts by weight per 100 parts by weight of polyvinylchloride, said outer layer being a skin (13) for the surface of said insulating layer (12) and having a thickness from 5 to 30% of the thickness of said insulating layer, the material constituting said skin containing a quantity of plasticizer from 10 to 40 parts by weight per 100 parts by weight of polyvinylchloride.

2. Low voltage cable according to claim 1, characterized by the fact that said mineral filler is calcium carbonate.

3. Low voltage cable according to claim 2, characterized by the fact that said calcium carbonate is added in a preferred proportion of 400 parts by weight per 100 parts by weight of polyvinylchloride.

4. Low voltage cable according to claim 1 characterized by the fact that said mineral filler is magnesium carbonate.

5. Low voltage cable according to claim 4, characterized by the fact that said magnesium carbonate is added in a preferred proportion of 400 parts by weight per 100 parts by weight of polyvinylchloride.

6. Low voltage cable according to any one of the preceding claims, characterized by the fact that the plasticizer in said material of said insulating layer is contained in a quantity of 100 parts by weight per 100 parts by weight of polyvinylchloride.

7. Low voltage cable according to any one of claims 1 to 6, characterized by the fact that said plasticizer is Di-2(ethyl-hexyl)-phthalate.

8. Low voltage cable according to any one of the preceding claims, characterized by the fact that in the material constituting said skin the plasticizer is comprised in a quantity of 30 parts by weight per 100 parts by weight of polyvinylchloride.

9. Low voltage cable according to claim 8, characterized by the fact that said plasticizer is Di-2-(ethyl-hexyl)-phthalate.

10. Low voltage cable according to any one of the preceding claims, characterized by the fact that the thickness of said skin is 15% of the insulating layer thickness.

## Patentansprüche

1. Niederspannungskabel welches einen Leiter hat, der durch einen oder mehrere miteinander verdrallte Drähte gebildet und mit einer Isolierschicht und einer äußeren umgebenden Lage bedeckt ist, wobei beide Lagen aus einem Material auf der Basis von Polyvinylchlorid (PVC) gebildet sind und wenigstens ein Plastifiziermittel enthalten, und wobei das Material für die Isolierlage weiterhin wenigstens einen Mineralfüllstoff enthält, dadurch gekennzeichnet, daß der Mineralfüllstoff in dem Material für die Isolierlage (12) in einem Anteil von 40 bis 500 Gewichtsteilen je 100 Gewichtsteile Polyvinylchlorid enthalten ist, das Plastifiziermittel in dem Material in einem Anteil von 60 bis 120 Gewichtsteilen je 100 Gewichtsteile Polyvinylchlorid enthalten ist, die äußere Lage eine Haut (13) für die Fläche der Isolierlage (12) ist und eine Dicke von 5 bis 30% der Dicke der Isolierlage hat, und das die Haut darstellende Material eine Menge an Plastifiziermittel von 10 bis 40 Gew.-Teile je 100 Gew.-Teile Polyvinylchlorid enthält.

2. Niederspannungskabel nach Anspruch 1, dadurch gekennzeichnet, daß der Mineralfüllstoff Kalziumcarbonat ist.

3. Neiderspannungskabel nach Anspruch 2, dadurch gekennzeichnet, daß das Kalziumcarbonat in einem bevorzugten Anteil von 400 Gew.-Teile je 100 Gew.-Teile Polyvinylchlorid zugegeben ist.

4. Niederspannungskabel nach Anspruch 1, dadurch gekennzeichnet, daß der Mineralfüllstoff Magnesiumcarbonat ist.

5. Niederspannungskabel nach Anspruch 4, dadurch gekennzeichnet, daß das Magnesiumcarbonat in einem bevorzugten Anteil von 400 Gew.-Teile je 100 Gew.-Teile Polyvinylchlorid zugegeben ist.

6. Niederspannungskabel nach irgendeinem der vorhergehenden Ansprüche, dadurch gekennzeichnet, daß das Plastifiziermittel in dem Material der Isolierlage in einer Menge von 100 Gew.-Teile je 100 Gew.-Teile Polyvinylchlorid enthalten ist.

7. Niederspannungskabel nach irgendeinem der Ansprüche 1 bis 6, dadurch gekennzeichnet, daß das Plastifiziermittel ein Di-2-(ethylhexyl)-phthalat ist.

8. Niederspannungskabel nach irgendeinem der vorhergehenden Ansprüche, dadurch gekennzeichnet, daß in dem die Haut bildenden Material das Plastifiziermittel in einer Menge von 30 Gew.-Teile je 100 Gew.-Teile Polyvinylchlorid enthalten ist.

9. Niederspannungskabel nach Anspruch 8, dadurch gekennzeichnet, daß das Plastifiziermittel Di-2-(ethylhexyl)-phthalat ist.

10. Niederspannungskabel nach irgendeinem der vorhergehenden Ansprüche, dadurch gekennzeichnet, daß die Dicke der Haut 15% der Dicke der Isolierlage beträgt.

## Revendications

1. Câble à bas voltag ayant un conducteur formé par un ou plusieurs fils torsadés ensemble et couvert par une couche isolante et une couche enveloppante externe, lesdites deux couches étant en matériau basé sur chlorure de polyvinyle (PVC) et contenant au moins un plastifiant, ledit matériau pour ladite couche isolante contenant aussi au moins un matériau de charge minéral, caractérisé en ce que ledit matériau de charge minéral est contenu dans le matériau pour la couche isolante (12) en une proportion de 40 à 500 parties en poids pour 100 parties en poids de chlorure de polyvinyle, que ledit plastifiant est contenue dans le matériau en une proportion de 60 à 120 parties en poids pour 100 parties en poids de chlorure de polyvinyle, ladite couche externe étant une peau (13) pour la surface de ladite couche isolante (12) et ayant une épaisseur de 5 à 30% de l'épaisseur de ladite couche isolante, ledit matériau formant ladite peau contenant une quantité de plastifiant de 10 à 40 parties en poids pour 100 parties en poids de chlorure de polyvinyle.

2. Câble à bas voltage suivant la revendication 1, caractérisé en ce que ledit matériau de charge minéral est du carbonate de calcium.

3. Câble à bas voltage suivant la revendication 2, caractérisé en ce que ledit carbonat de calcium est ajouté de préférence, en une proportion de 400 parties en poids pour 100 parties en poids de chlorure de polyvinyle.

4. Câble à bas voltage suivant la revendication 1, caractérisé en ce que ledit matériau de charge minéral est du carbonate de magnesium.

5. Câble à bas voltage suivant la revendication 4, caractérisé en ce que ledit carbonate de magnesium est ajouté, de préférence, en une proportion de 400 parties en poids pour 100 parties en poids de chlorure de polyvinyle.

6. Câble à bas voltage suivant une quelconque des revendications qui précèdent, caractérisé en ce que le plastifiant dans ledit matériau de ladite couche isolante est contenu en une quantité de 100 parties en poids pour 100 parties en poids de chlorure de polyvinyle.

7. Câble à bas voltage suivant une quelconque des revendications de 1 à 6, caractérisé en ce que ledit plastifiant est du Di-2-(éthyle-hexyle)-phtalate.

8. Câble à bas voltage suivant une quelconque des revendications qui précèdent, caractérisé en ce que dans le matériau formant ladite peau, le plastifiant est contenu en une quantité de 30 parties en poids pour 100 parties en poids de chlorure de polyvinyl.

9. Câble à bas voltage suivant la revendication 8, caractérisé en ce que ledit plastifiant est du Di-2-(éthyle-hexyle)-phtalat.

10. Câble à bas voltage suivant une quelconque des revendications qui précèdent, caractérisé en ce que l'épaisseur de ladite peau est 15% de l'épaisseur de la couche isolante.
